

1

3,462,271

## DIAZOTYPE MATERIAL

Herbert Rauhut and Oskar Süs, Wiesbaden-Biebrich, Germany, assignors, by mesne assignments, to Keuffel & Esser Company, Hoboken, N.J.  
No Drawing. Filed May 5, 1966, Ser. No. 547,738  
Claims priority, application Germany, May 8, 1965,  
K 56,060

The portion of the term of the patent subsequent  
to Sept. 13, 1983, has been disclaimed  
Int. Cl. G03c 1/54; C07c 113/00  
U.S. Cl. 96—91

11 Claims

## ABSTRACT OF THE DISCLOSURE

Diazotype material of improved stability and light sensitivity is provided through the use of p-phenylenediamine diazonium compounds which are meta-substituted with alkoxy substituents and which additionally bear a hydroxyalkyl substituent in the p-amino group.

The present invention relates to a diazotype material and more particularly relates to improved photosensitive diazo components useful in diazotype reproduction material.

In copying papers and other diazotype materials that have been sensitized with diazo compounds, the derivatives of unilaterally diazotized p-phenylenediamine have been used as the photosensitive components. These diazonium compounds have a tertiary amino group of basic character and they have been used successfully for both the dry process and the semiwet process.

For the dry process the diazo compounds which are most suitable are those containing lower alkyl groups attached to the basic nitrogen atom, while for the semiwet process the best ones are those in which the basic nitrogen atom is attached to higher hydrocarbon radicals.

The substituents on the basic nitrogen atom affect not only coupling speed, but they also affect the light sensitivity and keeping qualities of the diazo compounds and the light-sensitive layers prepared therewith.

In considerable measure the properties of the p-aminobenzene diazo compounds depend also on substituents attached to the phenylene ring. A substituent such as a methyl, methoxy or carboxyl group in a position ortho to the diazonium group, brings about a considerable improvement in stability and at the same time a color shift toward blue. Light sensitivity is, however, lowered by these substituents. The presence of an alkoxy group in a position meta to the diazonium group makes the diazo compound considerably more light sensitive in relation to the unsubstituted compound, but the keeping qualities become poorer as a result. Despite their poor stability, this type of diazo compound is nevertheless important because of its high light sensitivity and it finds practical use in cases where copies have to be prepared as quickly as possible.

It has been found that the stability of this general type of meta-substituted diazonium compounds can be improved without loss of light sensitivity through the use of heteroatom substituents in the alkoxy group in the position meta to the diazonium group. Some useful improvements in such diazonium compounds have been disclosed in related copending U.S. patent applications owned by the assignee of the present invention. U.S. application Ser. No. 311,220, filed Sept. 24, 1963, now U.S. Patent No. 3,272,630, describes a group of alkoxy-, aryloxy-, and tertiary amino-substituted 3-alkoxydiazonium compounds. Application Ser. No. 414,878, filed Nov. 30, 1964, now U.S. Patent No. 3,280,246 describes a group of alkylmercapto- and amino-substituted 3-alkoxy-

2

diazonium compounds. Application Ser. No. 425,921, filed Jan. 15, 1965, describes a group of alkoxy-, alkylmercapto- and amino-substituted 3-hydroxyalkoxydiazonium compounds. Application Ser. No. 547,721, filed May 5, 1966, describes a group of quaternary amino-substituted 3-alkoxydiazonium compounds.

Now, according to the present invention, there is provided diazotype material having improved stability and light sensitivity comprising substituted p-aminobenzene diazonium compounds which are meta-substituted with alkoxy, aryloxy, or aralkoxy groups and additionally by hydroxyalkyl substituent in the p-amino group. The light-sensitive diazonium compounds of the present invention have the general formula:



wherein

R is an alkylene group which contains at least 2 C-atoms,  
R<sub>1</sub> is an alkylene group,  
R<sub>2</sub> is an alkyl, aralkyl, or hydroxyalkyl,  
Z is an alkoxy, aralkoxy, aryloxy, or the group



wherein

R<sub>3</sub> is hydrogen, or an alkyl or hydroxyalkyl,  
R<sub>4</sub> is alkyl, hydroxyalkyl, or aralkyl, or  
R<sub>3</sub> and R<sub>4</sub>, together with the nitrogen, for an unsubstituted or substituted 5- or 6-membered heterocyclic group,  
X is hydrogen or a halogen or a methyl group, and  
Y is an anion of an acid.

The hydroxyalkyl radicals present in the diazo compounds defined above, including the hydroalkyl groups standing in some cases in place of the symbols R<sub>2</sub>, R<sub>3</sub> and R<sub>4</sub> used in the general formula, are preferably mono-hydroxyalkyl groups but may, however, also contain more than one hydroxyl group. Of the alkyl or alkylene radicals, radicals with up to four carbon atoms are preferred.

Where R<sub>2</sub> and R<sub>4</sub> are aralkyl groups, the benzyl group is preferred, which may optionally contain one or several low alkyl radicals or, on the nucleus, other substituents inert in the reaction.

The diazotype material according to the present invention exhibits particularly good stability with very good light sensitivity. The diazo compounds which characterize the material have good compatibility with additives and stabilizers such as, e.g., citric acid, thiourea, zinc chloride, naphthalene-1,3,6-trisulfonic acid. The material according to the invention can be prepared both as two-component material for the so-called dry process and as one-component material for the so-called semiwet process. Preferably, there are used for the dry process two-component material diazo compounds which at the amino group on the nucleus bear a low hydroxyalkyl radical besides a second such radical or a low alkyl radical and, for the semiwet process one-component material, diazo compounds which bear, at the amino group on the

nucleus, a higher alkyl or hydroxyalkyl or aralkyl radical as a substituent in addition to the hydroxyalkyl radical which is always necessary.

By the presence of hydroxyl groups at the alkali radicals which are attached to the amino group on the nucleus, solubility is increased compared with the compounds which have no hydroxyl group there. Moreover, the coupling dyes from the diazo compounds which are hydroxyalkylated at the amino nitrogen are, in general, not so sensitive to changes in pH value, are more bluish, and in continuous tones are of the same color as in the full shades.

It is observed that it is not advantageous to use diazo compounds in which all alkyl groups are hydroxylated. Apart from the fact that the solubility of the diazo compounds is so increased that they are difficult to precipitate and their preparation is therefore attended by difficulties, the water fastness of the coupling dyes formed from these compounds is unsatisfactory.

The diazo compounds which characterize the reproduction material according to the invention are new and are in general used as diazonium chloride in the form of the double salts with metal halides, for example zinc chloride or cadmium chloride. However, they may also be used in other precipitation forms, e.g., as sulfates, phosphates, borofluorides, for the preparation of the light-sensitive coatings.

Some of the present diazo compounds are shown in the table.

TABLE



The preparation of the diazo compounds according to the above general formula is effected according to methods which are known in the literature and which are also stated in the above-mentioned copending applications, but using for example hydroxylated alkyl halides instead of alkyl halides for the alkylation of the amino group on the nucleus. It has, however, proved expedient to effect the introduction of the hydroxyalkyl group into the amino group on the nucleus by alkylation with hydroxylated alkyl halides before introducing a higher alkyl group or an aralkyl group. If the amino group concerned is already substituted with an alkyl or aralkyl group, the hydroxyalkyl group is best introduced with the aid of alkylene oxide, e.g., ethylene oxide or propylene oxide. Other methods of preparation may also be effectively employed.

The present diazo compounds are used to prepare diazotype materials in the usual manner as typically shown in the examples. Dry or semiwet developing processes may be employed according to the material prepared and, depending upon the azo coupler components selected, dye images of various colors may be rapidly formed.

## EXAMPLE 1

In order to prepare diazotype paper, photocopying base paper of the usual kind which is provided with a precoat consisting of colloidal silicic acid and polyvinyl acetate is coated on the precoated surface with an aqueous solution which contains in 100 cc. of water:

|                                                                                                                                                            |       |    |      |
|------------------------------------------------------------------------------------------------------------------------------------------------------------|-------|----|------|
| Citric acid                                                                                                                                                | ----- | g  | 0.50 |
| Sodium naphthalene-1,3,6-trisulfonate                                                                                                                      | ----- | g  | 3.60 |
| Saponin                                                                                                                                                    | ----- | g  | 0.05 |
| Isopropanol                                                                                                                                                | ----- | cc | 5.00 |
| Zinc chloride double salt of the diazo compound from 1-amino - 4 - (hydroxyethylbenzyl)amino-3-[ $\beta$ -(methoxyethoxy)] - 6 - chlorobenzene (Formula I) | ----- | g  | 2.00 |

After drying, the sensitized base paper is imagewise exposed under a transparent original and developed with a solution which contains in each 100 cc. of water:

|                                       | G.  |    |
|---------------------------------------|-----|----|
| Borax                                 | 2.5 | 5  |
| Sodium carbonate                      | 3.0 |    |
| Sodium chloride                       | 2.0 |    |
| Thiourea                              | 5.0 |    |
| Sodium isopropylnaphthalene sulfonate | 0.1 |    |
| Resorcinol                            | 0.6 | 10 |
| Phloroglucinol                        | 0.6 |    |

High-contrast brown images on a white background are obtained.

If the base paper sensitized in the manner described above is treated, after exposure under an original, with a solution which contains in each 100 cc. of water:

|                                                   | G.    |    |
|---------------------------------------------------|-------|----|
| Phloroglucinol                                    | 0.330 |    |
| Trisodium citrate                                 | 9.600 | 20 |
| Sodium benzoate                                   | 2.420 |    |
| Adipic acid                                       | 1.975 |    |
| Sodium chloride                                   | 5.700 |    |
| Sodium salt of a dialkylnaphthalene sulfonic acid | 0.200 | 25 |

neutral black images on a white background are obtained. Continuous tones are also of the same hue as the full shades.

#### Example 2

A photocopying base paper of the kind commonly used in diazotype processes and having a precoat consisting of colloidal silicic acid and polyvinyl acetate is coated on the precoated side with a solution which contains in 100 cc. of water:

|                                                                                                                                                            | G.   |    |
|------------------------------------------------------------------------------------------------------------------------------------------------------------|------|----|
| Tartaric acid                                                                                                                                              | 10.0 |    |
| Boric acid                                                                                                                                                 | 3.0  |    |
| Thiourea                                                                                                                                                   | 2.5  |    |
| 7-hydroxynaphthimidazole                                                                                                                                   | 2.0  | 40 |
| Zinc chloride double salt of the diazo compound from 1-amino - 4 - (hydroxyethylbenzyl)amino-3-[ $\beta$ -(methoxy)ethoxy] - 6 - chlorobenzene (Formula I) | 1.93 |    |

After drying, the sensitized base paper is imagewise exposed under a transparent original and developed with ammonia. Bluish red lines on a white background are obtained.

The foregoing examples have been presented for the purpose of illustration and should not be taken to limit the scope of the present invention. It will be apparent that the described examples are capable of many variations and modifications—all such variations and modifications are to be included within the scope of the present invention as set forth in the appended claims.

What is claimed is:

1. Diazotype reproduction material comprising a support and a photosensitive composition coated thereon, said composition comprising a photosensitive diazonium compound having the general formula:



65

wherein:

R is an alkylene group having 2 to 4 carbon atoms or a beta-hydroxypropylene group;

R<sub>1</sub> is an alkylene group, having 2 to 4 carbon atoms; R<sub>2</sub> is an alkyl group having 1 to 3 carbon atoms, benzyl, or hydroxyalkyl group; Z is an alkoxy having 2 to 4 carbon atoms, phenoxy, benzyloxy, or the group



wherein R<sub>3</sub> is an alkyl having 1 to 3 carbon atoms, or hydroxyalkyl group, and R<sub>4</sub> is an alkyl having 1 to 3 carbon atoms, or benzyl;

X is hydrogen or a halogen or a methyl group; and Y is an anion of an acid.

2. Material according to claim 1 wherein said diazonium compound is the zinc chloride double salt of 2-chloro-4-(N-hydroxyethyl-N-benzyl)amino-5 - [beta - (methoxy)ethoxy]benzene diazonium chloride.

3. Material according to claim 1 wherein said diazonium compound is the zinc chloride double salt of 2-chloro-4-(N-beta-hydroxypropyl-N-benzyl)-amino-5-[beta - (methoxy)ethoxy]benzene diazonium chloride.

4. Material according to claim 1 wherein said diazonium compound is the zinc chloride double salt of 2-methyl-4-(N-hydroxyethyl-N-ethyl)amino-5-[delta-(N - methyl - N-benzylamino)butoxy]benzene diazonium chloride.

5. Material according to claim 1 wherein said diazonium compound is the zinc chloride double salt of 3-[beta-(butoxy)ethoxy]-4 - (N-beta - hydroxybutyl - N - methyl)aminobenzene diazonium chloride.

6. Material according to claim 1 wherein said diazonium compound is the zinc chloride double salt of 3-[gamma-(diethylamino)propoxy]-4-(N-hydroxyethyl - N - benzyl)aminobenzene diazonium chloride.

7. Material according to claim 1 wherein said diazonium compound is the zinc chloride double salt of 2-chloro-4-(N-hydroxyethyl-N-hydroxyethyl)amino-5-[beta - (phenoxy)ethoxy]benzene diazonium chloride.

8. Material according to claim 1 wherein said diazonium compound is the zinc chloride double salt of 3-[beta-(benzyloxy)ethoxy]-4-(N-hydroxyethyl - N - propyl)aminobenzene diazonium chloride.

9. Material according to claim 1 wherein said diazonium compound is the cadmium chloride double salt of 2-methyl-4-(N-hydroxyethyl-N-ethyl)amino-5-[gamma-(N - hydroxyethyl-N-propyl - amino)propoxy]benzene diazonium chloride.

10. Material according to claim 1 wherein said diazonium compound is the zinc chloride double salt of 3-[beta-hydroxy-gamma-(N-diethylamino)propoxy] - 4 - (N - hydroxyethyl-N-ethyl)aminobenzene diazonium chloride.

11. Material according to claim 1 wherein said diazonium compound is the zinc chloride double salt of 3-[beta-hydroxy-gamma-(N-diethylamino)propoxy] - 4 - (N - hydroxyethyl-N-benzyl)aminobenzene diazonium chloride.

#### References Cited

##### UNITED STATES PATENTS

|           |         |                  |          |
|-----------|---------|------------------|----------|
| 2,529,464 | 11/1950 | Von Glahn et al. | 96—91    |
| 2,552,354 | 5/1951  | Von Glahn et al. | 96—91    |
| 3,272,630 | 9/1966  | Rauhut et al.    | 96—91 XR |
| 3,281,246 | 10/1966 | Rauhut et al.    | 96—91    |

NORMAN G. TORCHIN, Primary Examiner

C. BOWERS, Assistant Examiner

U.S. Cl. X.R.

96—49; 260—141

UNITED STATES PATENT OFFICE  
CERTIFICATE OF CORRECTION

Patent No. 3,462,271

August 19, 1969

Herbert Rauhut et al.

It is certified that error appears in the above identified patent and that said Letters Patent are hereby corrected as shown below:

Column 1, line 71, "U. S. Patent No. 3,280,246" should read -- U. S. Patent No. 3,281,246 --.

Signed and sealed this 9th day of December 1969.

(SEAL)

Attest:

Edward M. Fletcher, Jr.

Attesting Officer

WILLIAM E. SCHUYLER, JR.

Commissioner of Patents